

Aug. 3, 1943.

E. M. WANAMAKER ET AL.

**2,325,723**

## PURIFICATION IN ELECTROWINNING OF MANGANESE

Filed Feb. 27, 1942



INVENTOR.  
Elmer M. Wanamaker  
and William D. Morgan, Jr.  
BY

*Safford, Scull & Burgess*  
ATTORNEYS

## UNITED STATES PATENT OFFICE

2,325,723

PURIFICATION IN ELECTROWINNING OF  
MANGANESE

Elmer M. Wanamaker and William D. Morgan,  
Jr., Knoxville, Tenn., assignors to Electro  
Manganese Corporation, Minneapolis, Minn.,  
a corporation of Delaware

Application February 27, 1942, Serial No. 432,692

2 Claims. (Cl. 204—105)

The invention relates to the electrowinning of manganese, more particularly the purification of electrolyte to be used as the catholyte.

In the electrowinning of manganese, the electrolyte is divided into anolyte and catholyte. Anolyte is continually withdrawn from the anolyte chamber and used for the extraction of manganese from manganese ore, the anolyte being thereby enriched in manganese. At the same time, however, impurities are introduced into the extract from the ore, among which iron, arsenic, antimony, nickel and cobalt may be mentioned. The iron, arsenic and antimony are commonly removed by oxidizing the iron to the ferric condition, following which and at a suitable pH, iron is precipitated, together with arsenic and antimony if a sufficient amount of iron was present in solution. Following the precipitation of the iron, ammonium sulfide is used as a reagent for the precipitation of other impurities, such as nickel, cobalt and copper, in the form of their sulfides. The nickel and cobalt precipitated in the form of a sulfide mud is separated by filtration or otherwise and the filtrate then goes to the catholyte chamber of the cell, thus completing the cycle of the movement and treatment of the electrolyte, beginning with the removal of anolyte from the anolyte chamber and ending with the introduction of catholyte into the catholyte chamber. This cycle is continuously repeated.

In the process following this cycle, on which the process of the present invention is an improvement, a large excess of ammonium sulfide over that theoretically necessary to precipitate the nickel, cobalt and other elements whose sulfides are insoluble in the given solution, is used. For example, to a batch of 32,000 liters of an electrolyte from which the iron, arsenic and antimony have been precipitated, containing 20 to 50 grams per liter of manganese as manganese sulfate, ammonium sulfate 140 to 180 grams per liter and which may have a pH of about 7.2 to 7.5, about 60 liters of a saturated solution of ammonium sulfide are added. The purpose of using this large excess of ammonium sulfide is to precipitate the nickel, cobalt, etc., as sulfides as completely as possible. Owing, however, to this large excess, substantial quantities of manganese sulfide are also precipitated.

The mud, which may contain as much as 5 percent of the manganese in the ore treated, is either discarded entirely or submitted to a process comprising treatment with sulphuric acid to recover the manganese as manganese sulphate and

the sulphur as ammonium sulfide by absorption of the  $H_2S$  evolved in aqua ammonia.

This process has certain disadvantages which it is the object of the present invention to overcome. The recovery of manganese from the mud is troublesome and expensive. The use of the large excess of ammonium sulfide represents an economic loss and in turn results in an excessive precipitation of manganese as sulfide in the mud. Moreover the purification which is the objective of the use of this large excess of ammonium sulfide is incomplete and this incomplete purification is reflected in the quality of the cathode deposit.

In addition to nickel and cobalt there are other 15 impurities the removal of which is desired and the effect of which is evidenced by the physical character of the deposit as a whole as distinguished from the presence of nickel and cobalt as metallic impurities in the deposit.

For example, one of the disadvantages is the 20 tendency of the deposit, during formation and deposition on the cathode, to peel or crack and in some instances to actually fall off in the catholyte chamber, in contrast to the desired character 25 of the deposit which is a coherent coating sufficiently adherent to the cathode to permit its removal with the cathode from the cell prior to the subsequent treatment of the cathode to separate the metallic manganese deposit. The precise 30 nature of these impurities has not been definitely established although it is believed that they are of a colloidal nature and therefore pass through the filter membrane. It is believed that they comprise colloidal silicates and compounds 35 of manganese, cobalt and nickel in dispersed form.

It has been discovered that the stated disadvantages can be largely if not wholly overcome by effecting the precipitation of the nickel, cobalt, etc., in each cycle in the presence of a large 40 excess of sulfide mud obtained in a previous cycle. For example, to the extract from which iron, arsenic, antimony and the like have been removed there may be added, at a pH of about 7.2 to 7.5, not only ammonium sulfide but also sulfide mud from the next preceding cycle and the precipitation of nickel and cobalt thereby effected in the presence of that mud. This process is then repeated in each succeeding cycle, substantially 45 the same body of mud being continuously reused in the successive treatments or cycles. Analyses indicate the possibility that the composition of this body of mud in these successive treatments progressively changes, the nickel and cobalt content progressively increas- 50 55

ing and the manganese content correspondingly decreasing. In such change in composition, a point might be reached at which the cobalt and nickel content of the mud reaches a value making possible the economical recovery of the nickel and cobalt from the mud. Furthermore, such a progressive decrease in manganese content would constitute in effect an automatic process of recovery whereby the manganese is transferred from the mud to the electrolyte thereby obviating, to the extent to which this occurs, any separate and independent step of recovering manganese from the mud. In order to avoid too great an accumulation of mud, a fractional part thereof may be removed in each precipitation and discarded or subjected to a process for the recovery of the manganese and other constituents therein. However since, except for this fractional portion, the mud is used over and over again, the loss of manganese in the event that the excess mud is discarded is greatly reduced and the expense and trouble of recovering manganese from the excess mud is also reduced. In addition and perhaps most important of all, the character of the cathode deposit is improved and it has been found that by proceeding in accordance with the present invention it is possible to constantly and uniformly obtain smooth adherent deposits free from the previously uncontrollable tendency to crack and flake off. It is to be noted that this phenomenon of peeling and flaking off is to be distinguished from the phenomenon of receding which occurs in the absence of adequate control over cathode potential.

The principles of the invention will be defined in the claims and a specific illustrative embodiment will be described in conjunction with the accompanying drawing showing diagrammatically a flow sheet illustrating steps in the process of the invention and apparatus which may be employed in practicing the same.

Anolyte having a composition of 10 to 18 grams per liter of manganese as manganese sulfate, about 140 to 180 grams per liter of ammonium sulfate and a pH of about 1 to 2 is withdrawn from the anolyte chamber 38 of the cell 40 and passed through line 1 to the ore extractor or digester 2 where, by agitation with suitable manganese ore, the concentration of manganese in the extract is raised to 20 to 50 grams per liter and the pH raised to about 2 to 5. The pH of the extract is adjusted to about 5.5 to 6.0 and air or other suitable oxidizing agent employed to oxidize the iron to the ferric condition and cause the precipitation thereof along with arsenic, antimony and the like. The precipitate is then filtered in the filter 4 and a volume of filtrate equal to about 32,000 liters is passed through the line 5 to the tank 6 where the pH is adjusted to about 7.2 to 7.5 as, for example, by the addition of ammonia added through the line 7. The contents of the tank 6 is then passed through the line 9 provided with valve 3 to the tank 17 in which is retained sulfide mud (from the previous purification) to level 21 in the tank, the quantity of mud being approximately that which would be obtained by adding 60 liters of 45% ammonium sulfide solution to 32,000 liters of iron-free extract. In addition, 15 liters of 45% ammonium sulfide are added to the contents of the tank 17 and the entire contents are then suitably agitated and then permitted to settle. A quantity of mud, in addition to that originally in the tank 17, is formed and is indicated by the level line 20. The supernatant liquid, together with the addi-

tional or excess sulfide mud precipitate caused by the addition of the 15 liters of ammonium sulfide are siphoned off through the riser 19, line 18 provided with valve 29 and line 31, and filtered in the filter press 32. The filtrate is passed through the line 35 to catholyte storage tank 41 and thence through the line 42 to the catholyte compartment 39 of the manganese electrowinning cell 40. The precipitate of excess sulfide mud filter cake from the filter 32 (corresponding to the 15 liters of ammonium sulfide) is then passed through the line 36 to the mud storage tank 37.

During the treatment of the contents of tank 17, another batch of 32,000 liters of extract is passed from tank 6 through lines 9 and 12 provided with valves 13 and 14 into treatment tank 23 and the treatment therein is the same as that described above in describing the treatment of the contents of tank 17, sulfide mud being initially supplied to tank 23 from mud storage tank 37 through line 45 and line 47 provided with valve 48 and thereafter maintained in said tank up to the level 25. The supernatant liquid together with excess mud up to the level 24 is withdrawn from tank 23 through riser 19A, lines 22 and 31 and filtered in filter 32, in the same manner as described in connection with tank 17.

It will thus be seen that in each of the tanks 17 and 23 a substantially constant quantity or volume of sulfide mud is maintained, indicated in the drawing by the level lines 21 and 25, respectively. The only portion of the sulfide mud which is withdrawn from these tanks is the increased quantity produced therein by the successive additions of ammonium sulfide (passed through line 15 provided with valves 16 and 16A) in the successive treatments.

The two tanks 17 and 23 alternate in their functions; that is, while extract is being purified in one tank purified supernatant liquor is being siphoned off from the companion tank and delivered to the catholyte storage tank 41, so that the catholyte storage tank is being continually replenished with purified catholyte. There is always available, therefore, one tank having a suitable body of mud therein into which to charge iron-free extract for purposes of purification. As many separate purification tanks as desired may be used.

Whereas in the process in respect of which the present invention is an improvement, it was necessary to employ about 60 liters of 45% ammonium sulfide for each successive batch of about 32,000 liters of iron-free extract, the present invention makes it possible to reduce the ammonium sulfide down to at least 15 liters; and whereas in said previous process it was necessary to discard the entire sulfide mud precipitate or work it up for recovery of manganese and other constituents, according to the present invention, except for the increment of sulfide mud removed as herein described, the said sulfide mud is used over and over again in each of the tanks 17 and 23 and the quantity of mud which it is necessary to work up for recovery purposes or discard is very greatly reduced. Finally and perhaps most important, the continuous reuse of the mud in the precipitation of nickel and cobalt effects such a purification of the electrolyte that the cathode deposit obtained therefrom is substantially free from the disadvantage of cracking and peeling. Although the precise mechanism by which the purifying effect of the mud is obtained is not fully known, it is believed that it exercises a

unique adsorptive effect or other physical-chemical action by which the colloidal impurities which are believed to contribute to the cracking and peeling of the manganese cathode deposit are removed.

Instead of ammonium sulfide, which is preferred, it is possible to use soluble sulfides in general.

We claim:

1. In a cyclical process for the purification of catholyte in the electrowinning of manganese in which ore is extracted with anolyte and the extract is treated to remove iron and then with ammonium sulfide to precipitate nickel and cobalt as sulfides, whereby a sulfide mud is obtained containing nickel sulfide, cobalt sulfide and manganese sulfide, the mud is separated from the solution and the latter is used as catholyte, the improvement which comprises precipitating cobalt and nickel sulfides by adding ammonium sulfide in the presence of sulfide mud obtained in a previous cycle, and thereby

forming an additional quantity of mud, the proportion of said mud obtained in a previous cycle being in excess of said additional quantity.

2. In a cyclical process for the purification of catholyte in the electrowinning of manganese in which ore is extracted with anolyte and the extract is treated to remove iron and then with a soluble sulfide to precipitate nickel and cobalt as sulfides, whereby a sulfide mud is obtained containing nickel sulfide, cobalt sulfide and manganese sulfide, the mud is separated from the solution and the latter is used as catholyte, the improvement which comprises precipitating cobalt and nickel sulfides by adding said soluble sulfide in the presence of sulfide mud obtained in a previous cycle, and thereby forming an additional quantity of mud, the proportion of said mud obtained in a previous cycle being in excess of said additional quantity.

ELMER M. WANAMAKER.  
WILLIAM D. MORGAN, JR.